

# UNITED STATES PATENT OFFICE.

JACQUES COENRAAD-HARTOGS, OF ARNHEM, NETHERLANDS.

## SPINNING VISCOSA.

No Drawing.

Application filed June 30, 1924. Serial No. 723,365.

To all whom it may concern:

Be it known that I, JACQUES COENRAAD HARTOGS, a subject of the Queen of the Netherlands, residing at Arnhem, Province of Guelderland, Kingdom of the Netherlands, have invented certain new and useful Improvements in Spinning Viscose, for which I filed an application in Germany, May 8, 1923, and of which the following 10 is a specification.

Known spinning baths for making artificial silk and other artificial textile fibres from viscose, generally consist in a mineral acid solution, with or without the addition 15 of salts; sulphuric acid is generally used but hydro-chloric acid has also been suggested.

The present invention is based on the discovery that a small quantity of nitric acid 20 added to a sulphuric acid spinning bath for viscose has a very favourable effect on the lustre and feel of the artificial silk.

The invention consists in spinning viscose 25 in a bath consisting of a dilute solution of sulphuric acid, with or without a salt or salts, and containing a small quantity of

nitric acid. A very small proportion of nitric acid in the bath suffices to produce a good effect, even an addition of 0.1 per cent of nitric acid showing its influence. 30 Under certain conditions dependent upon the degree of maturity and composition of the viscose and also on the maturity of the soda cellulose used, the proportion of added nitric acid may be increased, for instance 35 it may amount to 5 per cent.

What I claim is:

1. A process of making artificial silk or other artificial textile products which consists in spinning viscose in a bath of a 40 dilute solution of sulphuric acid containing between 0.1 per cent and 5 per cent of nitric acid.

2. A spinning bath for making artificial 45 silk and other artificial textile products consisting of a dilute solution of sulphuric acid containing between 0.1 per cent, and 5 per cent, of nitric acid.

In testimony whereof I affix my signature.

JACQUES COENRAAD HARTOGS.